

[54] CALK FOR GOLF SHOES

[75] Inventor: Yahyo Aoyama, Tokyo, Japan

[73] Assignee: Miyata Kinzoku Kogyo Kabushiki  
Kaisha, Tokyo, Japan

[22] Filed: Aug. 29, 1973

[21] Appl. No.: 392,747

[52] U.S. Cl..... 36/67 B

[51] Int. Cl..... A44b 21/00

[58] Field of Search ..... 36/67 R, 67 B, 2.5 AH,  
36/59; 12/146

## [56] References Cited

## UNITED STATES PATENTS

2,895,235 7/1959 Melchiona..... 36/67 B

3,423,855 1/1969 Kosono ..... 36/67 D

## FOREIGN PATENTS OR APPLICATIONS

673,399 6/1952 Great Britain ..... 36/67 D

*Primary Examiner*—Richard J. Scanlan, Jr.  
*Attorney, Agent, or Firm*—Woodhams, Blanchard and Flynn

## [57] ABSTRACT

A calk to be mounted on the sole of a golf shoe, wherein the central spindle is made of a semi-hard steel containing about 0.45 percent of carbon and only the portion of said central spindle projecting below the base plate thereof is made to have a high hardness by quenching.

6 Claims, 7 Drawing Figures



PATENTED AUG 13 1974

3,828,364

FIG. 1A



FIG. 1B



FIG. 2



FIG. 3



FIG. 4



FIG. 5



FIG. 6



## CALK FOR GOLF SHOES

## BACKGROUND OF THE INVENTION

## 1. Field of the Invention

The present invention relates to an improvement of a calk to be mounted on the sole of a golf shoe, and particularly it relates to an improvement of the central spindle of a calk.

## 2. Description of the Prior Art

The golf shoe is used in walking not only on the turf of a golf course but also on the concrete floor and metal board in the club house or the gravel roads within the golf course very frequently. Under such circumstances, the golf shoe in the prior art has been defective in that the calk mounted on the sole of it gets quickly worn down and rounded off to become useless as a spike.

With a view to minimizing this wear, there have hitherto been proposed various golf shoes such as employing a calk prepared by forming it with a mild steel and hardening thereafter in its entirety, or a calk prepared by hardening only the portion 1 of the central spindle as shown in the appended FIG. 1A, or a calk wherein only the tip 3 of the central spindle is provided inserted therein with the core 2 having high hardness as shown in FIG. 1B.

However, those calks in the prior art have all been defective in that, in the case of the calk made of mild steel and subjected to hardening in its entirety, the base plate portion is apt to break and fall off rendering it impossible to remove the central spindle from the sole, in the case of the calk of FIG. 1A wherein only the central spindle has been subjected to hardening, the thickness of the portion 1 having high hardness is not sufficient so that the calk is apt to quickly wear down by the tip of calk and the effect of the hardening cannot be much expected, and in the case of the calk of FIG. 1B wherein the core 2 having high hardness has been inserted in just the tip of the central spindle, the portion 3 made of iron to hold said core 2 is apt to wear down and the degree of wearing of this portion is especially high due to its poor thickness, said wearing of the portion 3 holding the core 2 causing the latter to slip out of the former, thereby making the calk useless. Not only that, inasmuch as said core 2 is usually made of an alloy of superhigh hardness such as tungsten carbide, it is expensive and not easy to work thereupon.

## SUMMARY OF THE INVENTION

The present invention is intended to make up for the foregoing defects of the calks in the prior art and to provide a calk having the hereunder described characteristic features. To be precise, one object of the present invention is to provide a calk wherein the central spindle consists of a semi-hard steel containing about 0.45 percent of carbon so as to prevent occurrence of troubles not only in cutting the male screw thread to be provided for the upper half of the central spindle but also in the working for fixing the central spindle onto the base plate by calking or stamping a trade mark and the like onto the lower end of the central spindle. Another object of the present invention is to provide a calk having a very high abrasion resistance and a lasting effect of spike through the process characterized by that, subsequent to the foregoing working upon the central spindle, the portion of the central spindle pro-

jecting below the base plate is red-heated up to more than about 900° C by a high-frequency heater and hardened by quenching thereafter to thereby prevent hardening of the base plate while imparting a high hardness to just the lower half of the central spindle.

## BRIEF DESCRIPTION OF THE DRAWINGS

In the appended drawings:

FIG. 1A is a front view of the vertical section of the first embodiment of a calk in the prior art to be mounted on the sole of a golf shoe;

FIG. 1B is a front view of the second embodiment of a calk — partly broken away — in the prior art to be mounted on the sole of a golf shoe;

FIG. 2 is a perspective view of the central spindle relevant to a calk according to the present invention;

FIG. 3 is a perspective view of the base plate relevant to the same calk as that in FIG. 2;

FIG. 4 is a perspective view of the same calk — as assembled — as that in FIG. 2;

FIG. 5 is a front view of the vertical section of the same assembled calk as that in FIG. 4; and

FIG. 6 is a plan view — as taken from the bottom side — of the same calk as that in FIG. 4.

## DETAILED DESCRIPTION OF THE INVENTION

Referring to the embodiment of the present invention shown in FIGS. 2, 3, 4, 5 and 6, a calk for the golf shoe under the present invention consists of the central spindle 10 and the base plate 20.

The central spindle 10 consists of a semi-hard steel containing about 0.45 percent of carbon, the upper end of said central spindle being provided with the male screw 11 for the purpose of fixing it onto the sole of golf shoe by screwing, the middle portion of said central spindle being formed into an elliptic shaft 12 thicker than said male screw 11 so as to fit in the elliptic central hole 21 of the base plate 20 and also being provided with the flange 13 formed beneath said elliptic shaft 12 so as to seat the base plate thereon, and the lower half 14 of said central spindle being formed into an inverted cone, so as to comprise a spike.

The base plate 20 is made of a mild steel plate and is shaped in the form of a slightly concave disc whose center is provided with said elliptic hole 21 where said elliptic shaft 12 of the central spindle 10 is supposed to fit in. In this connection, the small holes 22, 22 bored in this base plate on both sides of said elliptic hole 21 are for the purpose of putting two ends of a tool for driving the screw 11 at the time of mounting the calk on the sole of a shoe.

When the upper half of the central spindle 10 is fitted in the elliptic hole 21 of the base plate 20 from the bottom side of said plate, the elliptic shaft 12 fits exactly in said hole 21 and the base plate 20 is seated on the flange 13. Upon this, when two side edges 15, 15 of the elliptic shaft 12 projecting above the surface of the base plate 20 are calked on the base plate 20 in such a fashion as shown in FIG. 5, the central spindle 10 and the base plate 20 come to conjoin securely to be no longer detachable. As a calk according to the present invention is assembled as above and, by virtue of the elliptic hole 21 and the elliptic shaft 12, it never permits free rotation of the central spindle 10 relative to the base plate 20, it can be firmly fixed on the sole of a golf shoe by intensely turning the base plate 20.

The elliptic shaft 12 according to the present invention has a merit that it renders it possible to perform the work of calking or deforming same without inflicting any damage on the male screw 11, and the height of the elliptic shaft 12 is such that it just slightly exceeds the thickness of the base plate 20 and does not stick out of the level of the rim of the concave base plate 20.

According to a calk under the present invention as assembled as above, the trade mark is stamped on the surface of the lower end of the central spindle 10, the lower half or spike 14 of the central spindle 10 projecting below the base plate 20 is red-heated up to more than about 900° C by a high-frequency heater and cooled with water immediately thereafter to effect quenching. In the case of a semi-hard steel containing about 0.45 percent of carbon employed for the present invention, as a result of said quenching, a greater part of the tip of said lower half 14 as denoted by  $\alpha$  in FIG. 5 gets hardened to be possessed of a superb abrasion resistance. Accordingly, in the case where the present calk is applied to the sole of a golf shoe, the degree of wear thereof at the time of walking on gravel roads or concrete floors can be minimized and a lasting effect of spike can be expected.

In this connection, inasmuch as the exclusive application of high-frequency heating to the lower half 14 of the central spindle has no effect of quenching the base plate 20, there is no fear of causing the base plate 20 to harden or break. Besides, a semi-hard steel containing about 0.45 percent of carbon employed for the central spindle 10 facilitates such workings as cutting of the male screw 11, calking and stamping of the trade name 16 as long as it retains a normal mildness, and therefore, it not only is very convenient for the present invention in this respect but also renders it possible to produce a durable calk for the golf shoe economically.

What is claimed is:

1. In a calk for a golf shoe having a central spindle defining an upper threaded portion and a lower conical portion forming a spike, and an enlarged concave base plate surrounding a central portion of said spindle and fixed relative thereto, comprising the improvement wherein said spindle is of a semi-hard steel and is solid throughout the length thereof, only said spike being heat hardened, said spindle having the central portion

thereof formed with an elliptical cross section, said spindle also having a shoulder formed between said spike and said central portion of elliptical cross section, said base plate having a central opening of substantially elliptical shape, said base plate being seated on said shoulder with said central portion extending through said opening, said central portion having a thickness greater than the thickness of said plate, and the edges of said central portion being deformed downwardly over said base plate for fixedly and nonrotatably connecting said base plate to said spindle.

2. A calk according to claim 1, wherein the spindle is made from a semi-hard steel containing approximately 0.45 percent carbon, and the spike being hardened by heating only said spike to a temperature of at least 900° C and thereafter quenching the spike.

3. A method for forming a calk for a golf shoe having a central spindle defining an upper threaded portion and a lower conical portion defining a spike, and an enlarged base plate fixed to said spindle and surrounding a center portion thereof, comprising the steps of providing a solid shaftlike member formed of a mild steel containing approximately 0.45 percent carbon, forming a conical portion on the lower end of said member so as to define said spike, said spike being solid, providing an enlarged base plate having a central opening therethrough, positioning said base plate in surrounding relationship to a center portion of said member, fixedly connecting said base plate to said member by causing relative physical deformation between said base plate and said member, and hardening only said spike by heating said spike to a temperature of at least 900° C and then quenching said heated spike to harden same.

4. A method according to claim 3, wherein the hardening of said spike occurs after said base plate has been fixedly connected to said member.

5. A method according to claim 4, including the step of threading the upper portion of said member before hardening said spike.

6. A process according to claim 3, wherein said spike is hardened by heating same with a high frequency heater so as to heat only said spike to the desired temperature, and thereafter immediately water quenching said spike.

\* \* \* \* \*